# EUROPEAN PATENT SPECIFICATION

(11) **EP 0 726 968 B1**
(45) Date of publication and mention of the grant of the patent: **17.11.1999**
(21) Application number: 94922040.4
(22) Date of filing: 05.07.1994
(51) Int. Cl.: C23C 22/36

(54) **COMPOSITION AND PROCESS FOR TREATING TINPLATE AND ALUMINUM**
ZUSAMMENSETZUNG UND VERFAHREN ZUM BEHANDELN VON ZINN UND ALUMINIUM
COMPOSITION ET PROCEDE POUR TRAITER LE FER BLANC ET L'ALUMINIUM

(30) Priority: 05.07.1993 JP 16560193
(43) Date of publication of application: 21.08.1996
(73) Proprietor: HENKEL CORPORATION, Plymouth Meeting, PA 19462 (US)
(72) Inventor: AOKI, Tomoyuki, Kanagawa-ken 253 (JP); SHIMIZU, Akio, Isehara-shi, Kanagawa-ken 259-11 (JP); YOSHIDA, Masayuki, Asahi-ku, Yokohama-shi, Kanagawa-ken 241 (JP)
(74) Representative: Sanderson, Laurence Andrew
(86) International application number: US9407298
(87) International publication number: WO9502077

(56) References cited:
- EP-A- 0 178 020
- DE-A- 3 236 247
- FR-A- 2 347 459
- GB-A- 2 014 617
- GB-A- 2 131 052
- JP-A- 54 024 232
- US-A- 4 470 853
- US-A- 4 992 115
- US-A- 4 992 116
- US-A- 5 139 586
- CHEMICAL ABSTRACTS, vol. 90, no. 26, 25 June 1979 Columbus, Ohio, US; abstract no. 208761q, NIHON PARKERIZING: "Surface treatment of aluminum" page 303; column r; XP002001672
- CHEMICAL ABSTRACTS, vol. 91, no. 18, 29 October 1979 Columbus, Ohio, US; abstract no. 144331k, NIHON PARKERIZING: "Surface treatment of tin-plated steel" page 219; column l; XP002001673

## Description

The invention relates to a novel composition, usually called a "bath" hereinafter for brevity, and process that can be used to treat the surface of both aluminum Dl cans and tinplate Dl cans and that impart an excellent corrosion resistance and paint adherence to the surface of these cans prior to painting and/or printing them. "Aluminum Dl cans" and "tinplate Dl cans" refer to cans fabricated by the drawing and ironing, also called draw-ironing, of aluminum sheet and tin-plated steel sheet respectively.

Aluminum Dl cans and tinplate Dl cans have heretofore been treated with separate special purpose surface treatment baths. Baths for treating the surface of aluminum Dl cans are exemplified by the bath taught in Japanese Laid Open [Kokai or Unexamined] Patent Application Number Sho 52-131937 [131,937/1977]. The surface treatment bath taught therein is an acidic aqueous coating solution that has a pH of approximately 1.0 to 4.0 and that contains phosphate, fluoride, and zirconium and/or titanium. Treatment with that conversion treatment bath results in the formation of a highly paint-adherent, highly corrosion-resistant conversion film on the aluminum surface. The main components of this film are phosphate salt and zirconium oxide or titanium oxide.

Baths for treating the surface of tinplate Dl cans are exemplified by the teaching of Japanese Laid Open Patent Application Number Hei 1-100281 [100,281/1989]. That document concerns a conversion film-forming bath for the treatment of metal surfaces. The bath in that case has a pH of 2 to 6 and contains 1 to 50 g/L of phosphate ions, 0.2 to 20.0 g/L of oxyacid ions, 0.01 to 5.0 g/L of tin ions, and 0.01 to 5.0 g/L of condensed phosphate ions. Treatment with that conversion treatment bath results in the formation of a highly corrosion-resistant film on the surface of tinplate Dl cans. The main component of this film is tin phosphate.

JP-A-54068734 discloses a surface treatment of tin plated steel with a solution containing Ti and/or Zr, phosphate and a hydroxycarboxylic acid.

Japanese Patent Application Number JP-A-54024232 discloses the use of comparatively high concentrations of zirconium and/or titanium in the surface treatment of aluminum or its alloys. US Patent No. 4992115 discloses the surface treatment of aluminum or its alloys using vanadium or cerium ions together with zirconium, phosphate and fluorine ions.

A device known as a washer is generally used to treat the surface of Dl cans. The formed Dl cans are continuously treated with a degreasing composition and a conversion coating composition while turned upside down. Washers currently in use most often execute the following 6 processes: preliminary degreasing, degreasing, water wash, surface treatment, water wash, and a wash with de-ionized water.

In order to conduct surface treatment using such a washer, it has been necessary to select a surface treatment bath adapted to the type of Dl cans to be treated. In other words, a treatment bath in accordance with, for example, the invention in Japanese Laid Open Patent Application Number Sho 52-131937 would be used as the surface treatment bath for aluminum Dl cans, while a treatment bath in accordance with, for example, Japanese Laid Open Patent Application Number Hei 1-100281 would be used as the treatment bath for tinplate Dl cans.

Accompanying recent increases in the diversity of Dl can fabrication, there has been increasing opportunity to collect aluminum Dl cans and tinplate Dl cans into respective lots of some size and treat these in a single washer in an alternating sequence. However, a high-quality film with good corrosion resistance is not produced when the treatment bath in accordance with Japanese Laid Open Patent Application Number Sho 52-131937 is also applied to tinplate Dl cans. On the other hand, a conversion film is not formed when the treatment bath of Japanese Laid Open Patent Application Number Hei 1-100281 is also applied to aluminum Dl cans; this results in a poor corrosion resistance and a poor paint film adherence. As a result, each time the treatment substrate changes, it has been necessary to discard the treatment bath, clean the treatment chamber itself, and install a freshly prepared treatment bath that corresponds to the type of substrate.

In view of the circumstances described above, the present invention seeks to provide a multipurpose treatment bath and treatment process wherein a single treatment bath can be used to lay down a highly corrosion-resistant, highly paint-adherent film on the surface of both aluminum Dl cans and tinplate Dl cans.

The applicants have discovered that eluted metal ions, i.e., aluminum ions or tin ions, have a negative effect on film formation on the surface of a substrate which is not of the same metal. This is a major reason why a high-quality film is not formed when the conventional treatment baths are also applied to substrate different from the one for which they were designed. The applicants further formulated the following working hypotheses which were useful in solving the problems with the prior art as outlined above.
(1) With the conventional treatment baths, a film based on zirconium oxide or titanium oxide is formed on the surface of aluminum Dl cans, while a tin oxide-based film is formed on the surface of tinplate Dl cans.
(2) Etching of the metal substrate is necessary in order to form the films noted under (1), and this is most readily achieved by adjustment of the treatment bath pH to 2.0 to 4.0. At a pH below 2.0, film formation is impaired due to an excessive etch, while it becomes difficult to produce a highly corrosion-resistant film at a pH in excess of 4.0. Therefore, the pH should be controlled to 2.0 to 4.0.
(3) Tin ions (Sn²⁺, Sn⁴⁺) elute from the surface of tinplate Dl cans under the conditions noted in item (2). When an aluminum can is then treated, the divalent tin ions that have eluted into the treatment bath tend to be reduced to tin metal at the aluminum surface; this prevents the formation of a high-quality film on the aluminum surface. As a result, an oxidizing agent is preferably added to the treatment bath in order to rapidly oxidize the tin ions in the treatment bath to the tetravalent state and thereby achieve their stable presence in the bath.
(4) Aluminum ions elute from the aluminum surface under the conditions noted in item (2), and these aluminum ions destabilize any zirconium or titanium compounds present in the bath. To counter this, fluoride or hydrofluoric acid preferably is added to the treatment bath in order to stabilize the presence of aluminum in the treatment bath by forming fluoride complexes with the aluminum ions.
(5) While the oxidising agent accelerates the formation of zirconium oxide or titanium oxide on an aluminum surface, it tends to inhibit the formation of a protective coating including tin phosphate on a tin surface. Since more than 500 parts per million by weight (hereinafter usually abbreviated "ppm") of oxidising agent will usually prevent film formation, the appropriate upper limit on the oxidising agent is 500 ppm. Excessive levels of hydrofluoric acid or fluoride result in an excessive etch, which degrades the appearance, and a suitable upper limit on this additive is 2,000 ppm as fluorine.

According to one aspect of the present invention there is provided a process of treating tinplate and aluminum surfaces in order to form a protective coating thereon, in which the surfaces are contacted with an acidic aqueous liquid composition which has a pH value in the range of from 2.0 to 4.0 and besides water comprises the following components:
(A) at least one dissolved zirconium or titanium compound in an amount stoichiometrically equivalent to a total amount of zirconium and/or titanium in the range of from 10 to 200 ppm;
(B) hydrogen peroxide in an amount of from 20 to 500 ppm;
(C) one or more dissolved fluorine-containing anion(s) and/or corresponding acid(s), in an amount of from 10 to 2000 ppm stoichiometric equivalent as F⁻; and
(D) dissolved phosphate anions in an amount of at least 10 ppm; for such a time and at such a temperature as to form the desired protective coating.

The process of the invention can of course be applied to tinplate cans or aluminum cans, but it most truly achieves its objective when treatment is effected on a sequence of tinplate cans preceded and/or followed by aluminum cans.

Preferably, the contact time is in the range of from 2 to 120 seconds, and during contact the acidic aqueous liquid composition is maintained at a temperature in the range of from 20° to 65°C.

According to another aspect of the present invention there is also provided an acidic aqueous liquid composition for treating both aluminum and tinplate surfaces by the processes herein disclosed, so as to form a protective coating thereon, said composition comprising the components already indicated above.

A preferred composition also contains:
(E) an organic acid able to form complex ions with dissolved tin and/or aluminum ions.

Preferably the concentration of component (B) is from 40 to 200 ppm of hydrogen peroxide, the concentration of component (C) is from 20 to 900 ppm as F⁻, and the concentration of component (D) is from 10 to 500 ppm as phosphate. More preferably, the concentration of component (A) is from 10 to 150 ppm stoichiometric equivalent as the total of zirconium and titanium, the concentration of component (C) is from 40 to 500 ppm as F⁻, and the concentration of component (D) is from 20 to 90 ppm as phosphate. More preferably, the concentration of component (A) is from 20 to 100 ppm stoichiometric equivalent as the total of zirconium and titanium, and the concentration of component (C) is from 60 to 200 ppm as F⁻. Still more preferably, the concentration of component (A) is from 25 to 90 ppm stoichiometric equivalent as the total of zirconium and titanium, and the concentration of component (C) is from 90 to 165 ppm as F⁻.

Also preferred are compositions wherein component (A) is selected from the group consisting of fluozirconic and fluotitanic acids and salts thereof, and the pH is from 2.5 to 3.3.

Thus, the composition of this invention contains phosphate ion and at least 1 selection from zirconium compounds and titanium compounds and has a pH of 2.0 to 4.0, contains oxidising agent at no more than 500 ppm and at least 1 selection from simple and complex fluorides and their corresponding acids in a total amount that is no more than 2,000 ppm stoichiometric equivalent as fluorine. More preferably, the composition consists of water, the other ingredients noted above, and, if desired, the optional ingredient(s) noted below, and still more preferably consists only of these ingredients plus any necessary counterions to provide electrical neutrality to the composition, and of course possible impurities in the desired ingredients.

Hydrogen peroxide is present as oxidising agent in a composition according to the invention. Since the oxidising agent functions to stabilise the tin ion eluted from the Dl cans, its optimal content is a function of the amount of tin elution. An oxidising agent content in the range of 20 to 500 ppm is preferred for eluted tin concentration on the level of 50 ppm, while the range of 40 to 200 ppm for the oxidising agent is particularly preferred under most conditions of operation of a process according to this invention.

An organic acid that can readily form complexes with dissolved tin ions, aluminum ions, or both, for example, gluconic acid or oxalic acid, may be added on a supplementary basis in the event of a major decline in treatment bath stability due to metal ions, for example, iron or tin ions eluting from tinplate Dl cans, aluminum eluting from aluminum Dl cans, and the like.

The treatment bath must contain at least 1 selection from simple and complex fluorides and their corresponding acids. The fluoride content preferably is derived from hydrofluoric acid (HF) or a salt thereof such as sodium fluoride (NaF), or through the use of fluozirconic acid (H₂ZrF₆) or fluotitanic acid (H₂TiF₆) or their salts. The optimal fluoride content is determined as a function of the concentration of aluminum that elutes from the aluminum Dl cans. For example, 100 ppm aluminum preferably requires approximately 200 ppm fluorine. The fluoride content preferably falls in the range of 10 to 2,000 ppm as fluorine and more preferably, with increasing preference in the order given, falls in the range of 20 to 900, 40 to 500, 60 to 200 or 90 to 165, ppm as fluorine. When the fluoride content falls below 10 ppm as fluorine, the treatment bath becomes poorly reactive with the surface of aluminum Dl cans and an acceptable film is not usually produced.

The other components used in the invention treatment bath correspond to those used in conventional treatment baths. Thus, phosphoric acid (H₃PO₄) sodium phosphate (Na₃PO₄), and the like can be used to suppiy the phosphate ion in the treatment bath. Although less preferred, condensed phosphoric acids such as pyrophosphoric acid (H₄P₂O₇) and tripolyphosphoric acid (H₅P₃O₁₀) and their salts can also be used. While the phosphate ion content is not narrowly restricted, values in the range of 10 to 500 ppm are preferred and values in the range of 20 to 90 ppm are more preferred. In determining these values, the stoichiometric equivalent as phosphate of all phosphoric acid(s) and anions formed by ionisation thereof is considered to be phosphate.

The source of the zirconium and titanium compounds for the treatment bath is not narrowly restricted in scope, and the oxides, hydroxides, fluorides, and the like of zirconium and titanium can all be used, as can fluozirconic and fluotitanic acids and their salts, these acids and their salts being preferred. The content of zirconium and/or titanium compound must be from 10 to 200 ppm as Zr or Ti and more preferably, with increasing preference in order given, it will be from 10 to 150, from 20 to 100, or from 25 to 90 ppm as Zr or Ti.

The pH of the treatment bath can be adjusted through the use of an acid such as phosphoric acid, nitric acid, hydrochloric acid, or hydrofluoric acid, or through the use of an alkali such as sodium hydroxide, sodium carbonate, or ammonium hydroxide. The pH of the treatment bath normally should be from 2.0 to 4.0, while the range of 2.5 to 3.3 is preferred.

The technique for contacting the surface treatment bath with aluminum DI cans or tinplate DI cans is exemplified by immersion, spraying, and the like as generally known in the art, with spraying being the preferred technique. The temperature of the treatment bath should usually be 20º to 65ºC and is preferably 25º to 65º, more preferably 30º to 60º, or still more preferably 30º to 35ºC. The treatment time usually is from 2 to 120 seconds, preferably from 2 to 60 seconds, and particularly preferably from 15 to 60 seconds. A treatment time below 2 seconds does not usually produce an adequate reaction, thereby essentially precluding the formation of a highly corrosion-resistant film, while the improvement in performance diminishes at treatment times in excess of 60 seconds.

The treatment bath of the present invention is preferably used as part of the following process steps:
(1) cleaning of the Dl cans surface, preferably by degreasing;
(2) water wash;
(3) film-formation treatment, using a composition according to the invention;
(4) water wash;
(5) wash with deionized water; and
(6) drying.

### Examples

The usefulness of the surface treatment bath of the present invention is illustrated below through a comparison of several working examples with comparative examples. In these examples and comparison examples, any unspecified material in a treatment bath composition is water.

### General Conditions for Examples and Comparison Examples The aluminum Dl cans

The aluminum Dl cans were fabricated by the draw-ironing of aluminum sheet. They were cleaned using the hot aqueous solution of an acidic degreaser (Palklin™ 400, from Nihon Parkerizing Company, Ltd., Tokyo) and then subjected to surface treatment.

### The tinplate Dl cans

The tinplate Dl cans were fabricated by the draw-ironing of tin-plated steel sheet. They were cleaned using a hot aqueous solution of a weakly alkaline degreaser (Finecleaner™ 4361A, from Nihon Parkerizing Company, Ltd., Tokyo) and then subjected to surface treatment.

### Corrosion resistance

The corrosion resistance of the aluminum Dl cans was evaluated by immersing the treated cans in boiling water for 30 minutes and then evaluating the degree of blackening (the absence of blackening is preferred). The corrosion resistance of the tinplate Dl cans was evaluated using the iron exposure value ("IEV") measured in accordance with United States Patent Number 4,332,646. A lower IEV is indicative of a better corrosion resistance, and values at or below 150 are generally considered excellent.

### Paint adherence

The paint adherence was evaluated on the basis of the peel strength as follows: An epoxy-urea can paint was applied on the surface of the treated can to yield a paint film thickness of 5 to 7 micrometers. After baking for 4 minutes at 215° C, a 5 x 150 mm strip was cut from the can. A test specimen was prepared by hot-press bonding the strip with polyamide film, and the test specimen was peeled in a 180° peel test to provide the peel strength value. Higher peel strength values are indicative of a better paint adhesion, and values of at least 1.5 kilograms-force ("kgf")/5 mm of width are generally considered excellent.

### Example 1

Cleaned aluminum Dl cans and cleaned tinplate Dl cans were subjected to the following sequence of treatments: spraying for 30 seconds with surface treatment bath 1 heated to 40° C, then washing with tap water, spraying with de-ionized water (having a specific resistance of at least 3 megaohm-cm) for 10 seconds, and finally drying for 3 minutes in a forced convection drying oven at 180° C. The corrosion resistance and adherence of the resulting Dl cans were then measured.

### Surface treatment bath 1

| | |
|---|---|
| 75 % phosphoric acid (H₃PO₄) | 69 ppm (PO₄³⁻: 50 ppm) |
| 20 % fluozirconic acid (H₂ZrF₆) | 500 ppm (Zr⁴⁺: 44 ppm) |
| 20 % hydrofluoric acid (HF) | 210 ppm (total F⁻¹: 95 ppm¹) |
| 30 % hydrogen peroxide (H₂O₂) | 166 ppm (H₂O₂: 50 ppm) |
| pH 3.0 (adjusted with aqueous ammonia) | |

| | |
|---|---|
| ¹The total fluoride in this and all the other compositions containing both simple and complex fluoride ions is the total from both sources. | |

### Example 2

Cleaned aluminum Dl cans and cleaned tinplate Dl cans were subjected to the following sequence of treatments: spraying for 15 seconds with surface treatment bath 2 heated to 30° C, then a water wash, wash with de-ionized water, and drying as in Example 1. The corrosion resistance and adherence of the resulting DI cans were subsequently measured.

### Surface treatment bath 2

| | |
|---|---|
| 75 % phosphoric acid (H₃PO₄) | 69 ppm (PO₄³⁻: 50 ppm) |
| 20 % fluozirconic acid (H₂ZrF₆) | 1000 ppm (Zr⁴⁺: 88 ppm) |
| 20 % hydrofluoric acid (HF) | 210 ppm (total F⁻ 150 ppm) |
| 30 % hydrogen peroxide (H₂O₂) | 166 ppm (H₂O₂: 50 ppm) |
| pH 3.3 (adjusted with aqueous ammonia) | |

### Example 3

Cleaned aluminum Dl cans and cleaned tinplate Dl cans were subjected to the following sequence of treatments: spraying for 15 seconds with surface treatment bath 3 heated to 35° C, then a water wash, wash with deionized water, and drying as in Example 1. The corrosion resistance and adherence of the resulting Dl cans were subsequently measured.

### Surface treatment bath 3

| | |
|---|---|
| 75 % phosphoric acid (H₃PO₄) | 69 ppm (PO₄³⁻: 50 ppm) |
| 20 % fluotitanic acid (H₂TiF₆) | 500 ppm (Ti⁴⁺: 29 ppm) |
| 20 % hydrofluoric acid (HF) | 210 ppm (total F⁻: 110 ppm) |
| 30 % hydrogen peroxide (H₂O₂) | 664 ppm (H₂O₂: 200 ppm) |
| pH 2.5 (adjusted with aqueous ammonia) | |

### Example 4

Cleaned aluminum Dl cans and cleaned tinplate Dl cans were subjected to the following sequence of treatments: spraying for 30 seconds with surface treatment bath 4 heated to 40° C, then a water wash, wash with deionized water, and drying as in Example 1. The corrosion resistance and adherence of the resulting Dl cans were subsequently measured.

### Surface treatment bath 4

| | |
|---|---|
| 75 % phosphoric acid (H₃PO₄) | 138 ppm (PO₄³⁻: 100 ppm) |
| 20 % fluotitanic acid (H₂TiF₆) | 500 ppm (Ti⁴⁺: 29 ppm) |
| 20 % hydrofluoric acid (HF) | 210 ppm (total F⁻: 110 ppm) |
| 30 % hydrogen peroxide (H₂O₂) | 166 ppm (H₂O₂: 50 ppm) |
| pH 3.5 (adjusted with aqueous ammonia) | |

### Example 5

As discussed above, a critical issue for multipurpose treatment baths is the film performance when metal ions different from the substrate metal have entered the bath by a preceding elution from Dl cans. In this example, 500 ppm of tin ions was introduced into surface treatment bath 1 and the resulting surface treatment bath, heated to 60° C, was used for a 30-second spray treatment. Washing and drying were then carried out as in Example 1.

### Example 6

100 ppm of aluminum ions were introduced into surface treatment bath 1 and the resulting surface treatment bath, heated to 30° C, was used for a 30-second spray treatment. Washing and drying were then carried out as in Example 1.

### Example 7

50 ppm of tin ions were introduced into surface treatment bath 2 and the resulting surface treatment bath, heated to 60° C, was used for a 30-second spray treatment. Washing and drying were then carried out as in Example 1.

### Example 8

100 ppm of aluminum ions were introduced into surface treatment bath 2. and the resulting surface treatment bath, heated to 30° C, was used for a 30-second spray treatment. Washing and drying were then carried out as in Example 1, and the corrosion resistance and adherence of the resulting Dl cans were measured.

### Comparative Example 1

Cleaned aluminum Dl cans and cleaned tinplate Dl cans were subjected to the following sequence of treatments: spraying for 30 seconds with surface treatment bath 5 heated to 30° C, then a water wash, wash with deionized water, and drying as in Example 1. The corrosion resistance and adherence of the resulting Dl cans were subsequently measured.

### Surface treatment bath 5

| | |
|---|---|
| 75 % phosphoric acid (H₃PO₄) | 69 ppm (PO₄³⁻: 50 ppm) |
| 20 % fluozirconic acid (H₂ZrF₆) | 500 ppm (Zr⁴⁺: 44 ppm) |
| 20 % hydrofluoric acid (HF): | 210 ppm (total F⁻: 95 ppm) |
| pH 3.0 (adjusted with aqueous ammonia) | |

### Comparative Example 2

Cleaned aluminum Dl cans and cleaned tinplate Dl cans were subjected to the following sequence of treatments: spraying for 30 seconds with surface treatment bath 6 heated to 30° C, then a water wash, wash with deionized water, and drying as in Example 1. The corrosion resistance and adherence of the resulting Dl cans were subsequently measured.

### Surface treatment bath 6

| | |
|---|---|
| 75 % phosphoric acid (H₃PO₄) | 69 ppm (PO₄³⁻: 50 ppm) |
| 20 % hydrofluoric acid (HF) | 210 ppm (F⁻: 40 ppm) |
| pH 3.0 (adjusted with aqueous ammonia) | |

### Comparative Example 3

50 ppm of tin ions were introduced into surface treatment bath 5 and the resulting surface treatment bath, heated to 30° C, was used for a 30-second spray treatment. Washing and drying were then carried out as in Example 1, and the corrosion resistance and adherence of the resulting Dl cans were measured.

### Comparative Example 4

Cleaned aluminum Dl cans and cleaned tinplate Dl cans were subjected to the following sequence of treatments: heating a commercial surface treatment bath intended for application to aluminum Dl cans (Alodine™ 404, from Nihon Parkerizing Company, Ltd., Tokyo) to 30° C and spraying with this for 30 seconds, then a water wash, wash with deionized water, and drying as in Example 1. The corrosion resistance and adherence of the resulting Dl cans were subsequently measured.

### Comparative Example 5

Cleaned aluminum Dl cans and cleaned tinplate Dl cans were subjected to the following sequence of treatments: heating a commercial surface treatment bath intended for application to tinplate Dl cans (Palfos™ K3482, from Nihon Parkerizing Company, Ltd., Tokyo) to 30° C and spraying with this for 30 seconds, then a water wash, wash with deionized water, and drying as in Example 1. The corrosion resistance and adherence of the resulting Dl cans were subsequently measured.

The results of all the measurements noted above are shown in Table 1 on the following page.

### Benefits of the Invention

The treatment bath in accordance with the present invention produces a titanium oxide-containing or zirconium oxide-containing film on the surface of aluminum Dl cans and produces a tin oxide-containing film on the surface of tinplate Dl cans. This multipurpose applicability to different types of substrates is made possible by the presence in the treatment bath of both an oxidizing agent and hydrofluoric acid and/or fluoride and by the stipulation of specific upper limits for them. A process according to the invention provides cans, prior to painting and/or printing them, with an excellent corrosion resistance and paint adherence through a low-temperature treatment.

## Claims

1. A process of treating tinplate and aluminum surfaces in order to form a protective coating thereon, in which the surfaces are contacted with an acidic aqueous liquid composition which has a pH value in the range of from 2.0 to 4.0 and besides water comprises the following components:
(A) at least one dissolved zirconium or titanium compound in an amount stoichiometrically equivalent to a total amount of zirconium and/or titanium in the range of from 10 to 200 ppm;
(B) hydrogen peroxide in an amount of from 20 to 500 ppm;
(C) one or more dissolved fluorine-containing anion(s) and/or corresponding acid(s), in an amount of from 10 to 2000 ppm stoichiometric equivalent as F⁻; and
D) dissolved phosphate anions in an amount of at least 10 ppm; for such a time and at such a temperature as to form the desired protective coating.

2. A process as claimed in claim 1, in which the treatment is effected on a sequence of tinplate cans preceded and/or followed by aluminum cans.

3. A process as claimed in claim 1 or claim 2, where the contact time is in the range of from 2 to 120 seconds, and during contact the acidic aqueous liquid composition is maintained at a temperature in the range of from 20° to 65°C.

4. An acidic, aqueous liquid composition, suitable for treating both aluminum and tinplate surfaces by the process claimed in any of the preceding claims so as to form a protective coating thereon, which acidic composition has a pH value in the range of from 2.0 to 4.0 and besides water comprises the following components:
(A) at least one dissolved zirconium or titanium compound in an amount stoichiometrically equivalent to a total amount of zirconium and/or titanium in the range of from 10 to 200 ppm;
(B) hydrogen peroxide in an amount of from 20 to 500 ppm;
(C) one or more dissolved fluorine-containing anion(s) and/or corresponding acid(s), in an amount of from 10 to 2000 ppm stoichiometric equivalent as F⁻; and
(D) dissolved phosphate anions in an amount of at least 10 ppm.

5. An acidic aqueous liquid composition as claimed in claim 4, which also contains:
(E) an organic acid able to form complex ions with dissolved tin and/or aluminum ions.

6. An acidic aqueous liquid composition as claimed in claim 4 or claim 5, which apart from:
(F) dissolved aluminum ions, and/or
(G) dissolved tin ions
and perhaps impurities consists solely of water and the specified components (A)-(D) and optionally (E).

7. An acidic aqueous liquid composition as claimed in any of claims 4 to 6, wherein the concentration of component (B) is from 40 to 200 ppm of hydrogen perioxide, the concentration of component (C) is from 20 to 900 ppm as F⁻, and the concentration of component (D) is from 10 to 500 ppm as phosphate.

8. An acidic aqueous liquid composition as claimed in claim 7, wherein the concentration of component (A) is from 10 to 150 ppm stoichiometric equivalent as the total of zirconium and titanium, the concentration of component (C) is from 40 to 500 ppm as F⁻, and the concentration of component (D) is from 20 to 90 ppm as phosphate.

9. An acidic aqueous liquid composition as claimed in claim 8, wherein the concentration of component (A) is from 20 to 100 ppm stoichiometric equivalent as the total of zirconium and titanium, and the concentration of component (C) is from 60 to 200 ppm as F⁻.

10. An acidic aqueous liquid composition as claimed in claim 9, wherein the concentration of component (A) is from 25 to 90 ppm stoichiometric equivalent as the total of zirconium and titanium, and the concentration of component (C) is from 90 to 165 ppm as F⁻.

11. An acidic aqueous liquid composition as claimed in any of the preceding claims, wherein component (A) is selected from the group consisting of fluozirconic and fluotitanic acids and salts thereof, and the pH is from 2.5 to 3.3.

## Patentansprüche

1. Verfahren zur Behandlung von Zinnblech- und Aluminium-Oberflächen, um darauf eine Schutzbeschichtung zu bilden, worin die Oberflächen mit einer sauren, wäßrigen, flüssigen Zusammensetzung im Kontakt gebracht werden, die einen pH im Bereich von 2,0 bis 4,0 hat und neben Wasser die folgenden Komponenten umfaßt:
(A) wenigstens eine gelöste Zirconium- oder Titan-Verbindung in einer Menge im Bereich von 10 bis 200 ppm, die der Gesamtmenge von Zirconium und/oder Titan stöchiometrisch äquivalent ist;
(B) Wasserstoffperoxid in einer Menge von 20 bis 500 ppm;
(C) ein gelöstes, fluorenthaltendes Anion und/oder eine entsprechende Säure oder mehrere gelöste, fluorenthaltende Anionen und/oder entsprechende Säuren, in einer Menge von 10 bis 2000 ppm, die F⁻ stöchiometrisch äquivalent ist, und
(D) gelöste Phosphatanionen in einer Menge von wenigstens 10 ppm während einer solchen Zeitspanne und bei einer derartigen Temperatur, daß sich die erwünschte Schutzbeschichtung bildet.

2. Verfahren gemäß Anspruch 1, worin die Behandlung auf einer Reihe von Zinnblechdosen durchgeführt wird, denen Aluminiumdosen vorangingen und/oder folgten.

3. Verfahren gemäß den Ansprüchen 1 oder 2, worin die Kontaktzeit im Bereich von 2 bis 120 Sekunden liegt und während des Kontakts die saure, wäßrige, flüssige Zusammensetzung bei einer Temperatur im Bereich von 20 bis 65 °C gehalten wird.

4. Saure, wäßrige, flüssige Zusammensetzung, die zur Behandlung von sowohl Aluminium- als auch Zinnblech-Oberflächen durch das Verfahren geeignet ist, welches gemäß irgendeinem der vorhergehenden Ansprüche beansprucht wird, um somit auf denselben eine Schutzbeschichtung zu bilden, wobei die saure Zusammensetzung einen pH im Bereich von 2,0 bis 4,0 hat und neben Wasser die folgenden Komponenten umfaßt:
(A) wenigstens eine gelöste Zirconium- oder Titan-Verbindung in einer Menge im Bereich von 10 bis 200 ppm, die der Gesamtmenge von Zirconium und/oder Titan stöchiometrisch äquivalent ist;
(B) Wasserstoffperoxid in einer Menge von 20 bis 500 ppm;
(C) ein gelöstes, fluorenthaltendes Anion und/oder eine entsprechende Säure oder mehrere gelöste, fluorenthaltende Anionen und/oder entsprechende Säuren, in einer Menge von 10 bis 2000 ppm, die F⁻ stöchiometrisch äquivalent ist, und
(D) gelöste Phosphatanionen in einer Menge von wenigstens 10 ppm.

5. Saure, wäßrige, flüssige Zusammensetzung gemäß Anspruch 4, die auch
(E) eine organische Säure enthält, welche befähigt ist, mit gelösten Zinn- und/oder Aluminiumionen Komplexionen zu bilden.

6. Saure, wäßrige, flüssige Zusammensetzung gemäß den Ansprüchen 4 oder 5, welche, abgesehen von
(F) gelösten Aluminiumionen und/oder
(G) gelösten Zinnionen
und vielleicht Verunreinigungen nur aus Wasser und den vorgegebenen Komponenten (A) - (D) und gegebenenfalls (E) besteht.

7. Saure, wäßrige, flüssige Zusammensetzung gemäß den Ansprüchen 4 bis 6, worin die Konzentration der Komponente (B) 40 bis 200 ppm Wasserstoffperoxid beträgt, die Konzentration der Komponente (C) als F⁻ 20 bis 900 ppm beträgt, und die Konzentration der Komponente (D) als Phosphat 10 bis 500 ppm beträgt.

8. Saure, wäßrige, flüssige Zusammensetzung gemäß Anspruch 7, worin die Konzentration der Komponente (A) 10 bis 150 ppm beträgt, die dem gesamten Zirconium und Titan stöchiometrisch äquivalent ist, die Konzentration der Komponente (C) als F⁻ 40 bis 500 ppm ist, und die Konzentration der Komponente (D) als Phosphat 20 bis 90 ppm beträgt.

9. Saure, wäßrige, flüssige Zusammensetzung gemäß Anspruch 8, worin die Konzentration der Komponente (A) 20 bis 100 ppm beträgt, die dem gesamten Zirconium und Titan stöchiometrisch äquivalent ist, und die Konzentration der Komponente (C) als F⁻ 60 bis 200 ppm beträgt.

10. Saure, wäßrige, flüssige Zusammensetzung gemäß Anspruch 9, worin die Konzentration der Komponente (A) 25 bis 90 ppm beträgt, die dem gesamten Zirconium und Titan stöchiometrisch äquivalent sind, und die Konzentration der Komponente (C) als F⁻ 90 bis 165 ppm beträgt.

11. Saure, wäßrige, flüssige Zusammensetzung gemäß irgendeinem der vorhergehenden Ansprüche, worin die Komponente (A) aus der aus Fluorzirconium- und Fluortitansäure und deren Salzen bestehenden Gruppe ausgewählt ist und der pH 2,5 bis 3,3 beträgt.

## Revendications

1. Procédé pour le traitement de surfaces d'aluminium et de plaques d'étain pour y former un revêtement protecteur, procédé dans lequel les surfaces sont mises en contact avec une composition liquide aqueuse acide ayant une valeur de pH dans la plage de 2,0 jusqu'à 4,0 et en outre, l'eau comprend les composants suivants:
(A) au moins un composé titane ou zirconium dissous dans une quantité stoechiométriquement équivalente à une quantité totale de zirconium et/ou de titane dans la plage de 10 à 200 ppm ;
(B) du peroxyde d'hydrogène dans une quantité de 20 à 500 ppm ;
(C) un ou plusieurs anions contenant du fluor dissous et/ou des acides correspondants dans une quantité de 10 à 2000 ppm équivalents stoechiométriques en tant que F⁻ ; et
(D) des anions phosphates dissous dans une quantité d'au moins 100 ppm pour une durée à une température telles à former le revêtement protecteur souhaité.

2. Procédé selon la revendication 1, dans lequel le traitement est effectué sur une séquence de boîtes réalisée à partir de plaques d'étain précédée et ou suivie de boîtes d'aluminium.

3. Procédé selon la revendication 1 ou la revendication 1, dans lequel le temps de contact se situe dans la plage de 2 à 120 secondes et pendant le contact, la composition liquide aqueuse acide est maintenue à une température dans la plage de 20 à 65°C.

4. Composition liquide aqueuse acide convenant au traitement aussi bien des surfaces d'aluminium que des surfaces de plaques d'étain par le procédé revendiqué dans l'une quelconque des revendications précédentes de façon à y former un revêtement protecteur, laquelle composition a une valeur de pH dans la plage de 2.0 à 4.0 et en outre, l'eau comprend les composants suivants :
(A) au moins un composé titane ou zirconium dissous dans une quantité stoechiométriquement équivalente à une quantité totale de zirconium et/ou de titane dans la plage de 10 à 200 ppm ;
(B) peroxyde d'hydrogène dans une quantité de 20 à 500 ppm ;
(C) un ou plusieurs anions contenant du fluor dissous et/ou des acides correspondants dans une quantité de 10 à 2000 ppm équivalence stoechiométrique en tant que F⁻; et
(D) anions de phosphate dissous dans une quantité d'au moins 10 ppm.

5. Composition liquide aqueuse acide selon la revendication 4 qui contient également :
(E) un acide organique pouvant former des ions complexes avec des ions d'aluminium et/ou d'étain dissous.

6. Composition liquide aqueuse acide selon la revendication 4 ou la revendication 5, qui en plus des :
(F) ions aluminium dissous et/ou
(G) ions étain dissous
et éventuellement des impuretés, est exclusivement constituée d'eau et des composants spécifiques (A)-(D) et facultativement (E).

7. Composition liquide aqueuse acide selon l'une quelconque des revendications 4 à 6, dans laquelle la concentration du composant (B) est de 40 à 200 ppm de perioxyde d'hydrogène, la concentration du composant (C) est de 20 à 900 ppm en tant que F⁻, et la concentration du composant (D) est de 10 à 500 ppm en tant que phosphate.

8. Composition liquide aqueuse acide selon la revendication 7, dans laquelle la composition du composant (A) est de 10 à 150 ppm équivalence stoechiométrique en tant que total de zirconium et de titane, la concentration du composant (C) est de 40 à 500 ppm en tant que F⁻, et la concentration du composant (D) est de 20 à 90 ppm en tant que phosphate.

9. Composition liquide aqueuse acide selon la revendication 8, dans laquellc la concentration du composant (A) est de 20 à 100 ppm équivalence stoechiométrique en tant que total de zirconium et de titane et la concentration du composant (C) est de 60 à 200 ppm en tant que F⁻.

10. Composition liquide aqueuse acide selon la revendication 9, dans laquelle la concentration du composant (A) est de 25 à 90 ppm équivalence stoechiométrique en tant que total de zirconium et de titane, et la concentration du composant (C) est de 90 à 165 ppm en tant que F⁻.

11. Composition liquide aqueuse acide selon l'une quelconque des revendications précédentes, dans laquelle le composant (A) est choisi dans le groupe constitué par des acides fluozirconique et fluotitanique et leurs sels et le pH est de 2,5 à 3,3.
